

# United States Patent

Patrie

[15] 3,664,932

[45] May 23, 1972

[54] **OBJECTS OF ALUMINUM AND ALLOYS  
OF ALUMINUM HAVING COLORED  
COATINGS AND PROCESS**

[72] Inventor: **Jos Patrie**, Grenoble, France

[73] Assignee: **Cegedur GP**, Paris, France

[22] Filed: **Dec. 3, 1969**

[21] Appl. No.: **881,846**

[30] **Foreign Application Priority Data**

Dec. 6, 1968 France.....176899

[52] U.S. Cl. ....**204/35 N, 204/58**

[51] Int. Cl. ....**C23j 5/50**

[58] **Field of Search**.....**204/35 N, 38, 58, 42**

[56] **References Cited**

UNITED STATES PATENTS

3,382,160 5/1968 Asada .....204/35 N

*Primary Examiner*—John H. Mack

*Assistant Examiner*—Regan J. Fay

*Attorney*—McDougall, Hersh & Scott

[57]

**ABSTRACT**

The process for providing colored coatings on aluminum and alloys of aluminum in which the surface is first anodized to form a porous layer and colored particles of metal compound are deposited in the porous layer by alternating current electrolysis with the object mounted as an electrode in an electrolyte containing the salt of the metal, and then subjecting the deposited particles to dissolution by mounting the object as an anode for direct or rectified current electrolysis until a color of the desired value is secured.

18 Claims, No Drawings

**OBJECTS OF ALUMINUM AND ALLOYS OF ALUMINUM  
HAVING COLORED COATINGS AND PROCESS**

This invention relates to aluminum and alloys of aluminum having a colored protective coating and methods for preparation of same.

Numerous processes are available for use in producing a colored coating on the surface of anodized aluminum and alloys thereof. In the French Pat. No. 880,095, description is made of a coloring process comprising depositing particles of metal compound into the pores of a layer formed by anodization and while under alternating current electrolysis. The layer that is obtained is dark in color, depending somewhat upon the time of alternating current electrolysis. As a result, it has been the practice to terminate electrolysis when the desired color has been obtained and then seal the layer in boiling water. This process is subject to a serious disadvantage in that, at the start of the electrolysis, the deposit is non-uniform with the result that a non-uniform color is obtained.

It is an object of this invention to produce and to provide a process for producing a highly uniform clear color on an anodized layer of aluminum and in which the color is capable of being reproduced.

The process of this invention comprises restoring, by anodic dissolution, the clear colors observed during the initial stages of deposition, after a dark or black color effect has been obtained on the object formed of aluminum or alloys thereof, due to the presence of metal or metal compound particles in the pores of the formed layer of alumina. During anodic dissolution, the color turns clear as the treatment progresses and, contrary to what is observed in electrolytic coloring, the color rapidly becomes uniform over the entire surface of the object. In addition, the anodic dissolution treatment is highly flexible and thus gives more latitude for regulating the production parameters. This is highly advantageous insofar as commercial operation is concerned.

The following will briefly describe the practice of this invention for producing a colored layer on aluminum or alloy of aluminum. For this purpose, the object is initially anodized, such as in a sulphuric acid bath, to provide the object with a porous layer of alumina. Colored particles of a metal or metal compound are then deposited by electrolysis into the pores of the anodized layer, using a bath containing a dissolved salt of the constituent metal of the particles, giving a dark color effect. The electrolysis is operated with alternating current with the object to be coated forming one of the electrodes, while the other electrode, referred to as the counter-electrode, is made either of the constituent metal of the salt dissolved in the electrolyte or of a material which is resistant to the effect of the bath and which does not give rise to any secondary reactions during the electrolysis, such for example as stainless steel.

This is followed by anodic dissolution, in accordance with the practice of this invention. The object to be coated, which has a dark color or even a black color due to the presence of an excess of colored particles in the pores of the alumina layer, is mounted as an anode in a continuous current or direct current electrolysis cell. It is believed that the anion of the electrolyte combines with the metal compound deposited in the pores of the alumina layer to form a soluble salt of the metal. Anodic dissolution is accompanied by a lightening and standardization of the color due to the decrease and probably to the standardization of the thickness of the deposit. The operation is terminated by cutting the current when the required color has been obtained.

In a preferred embodiment of the invention, the dissolution stage is carried out in the same bath and in the same cell as the deposition by electrolysis. It is sufficient, for this purpose, to provide a switching device by which it is possible to change from alternating current to direct current. More simply, it is sufficient to provide a diode or a diode bridge in the circuit for converting the alternating current into a rectified unfiltered current which gives the same results as the direct current.

The electrolyte comprises an acid solution, and preferably a sulphuric acid solution, of a salt of a metal such as copper,

nickel, cadmium, cobalt, etc. The concentration of metal salts dissolved in the electrolyte may range from 0.15 g/liter to an amount to provide a saturated solution. The operation is carried out at bath temperature within the range of 5°-30° C and preferably of about room temperature, either at a constant current density of less than 5 A/dm<sup>2</sup> and preferably at a current density within the range of 0.1 to 2 A/dm<sup>2</sup>, or at a constant voltage within the range of 10 to 50 volts and preferably 15 to 25 volts for a period of from 10 seconds to 30 minutes, and generally from 1/2 to 15 minutes. While it is preferred to carry out anodic dissolution in the same electrolyte as for deposition by electrolysis, preferably under the same temperature conditions, use can be made of a different bath of a buffered sulphuric acid or salt thereof of corresponding pH.

15 The final colored layer can be fixed by any conventional process, such as by sealing in boiling water, varnishing or the like.

20 The color obtained is governed by the nature of the metal and the color intensity is governed both by the current density and by the duration of the anodic dissolution for the same initial color effect. For example, a wide range of reds from pink to deep scarlet, including copper shades, can be obtained with an electrolyte containing copper salts. The salts of nickel, cadmium or cobalt enable browns or gold hues to be obtained.

25 The final appearance is somewhat related to the surface quality of the object before the porous layer of alumina is formed. For example, on a brilliant or glossy surface, the color effects obtained by the process are brilliant while on a dull or mat surface, a dull or mat color will be secured. Accordingly, 30 it is advantageous to modify the surface characteristics of the object before coating. Such surface changes can be effected by conventional or known means including polishing, buffing, glazing, and the like, depending upon the finish required. For example, a mat finish is obtained by cleaning the object for 10 minutes at 50° C in a soda solution having a concentration of 50 g/liter, after which it is washed in a stream of water followed by immersion in nitric acid (36° Be) and then by further rinsing in a stream of water. The glossy or shiny finish is obtained by mechanical polishing or by chemical or electrolytic glossing.

35 The following examples are given by way of illustration, but not by way of limitation, of the practice of this invention.

40 In the following examples the objects are subjected to the following general steps:

45 surface preparation by one of the processes referred to above;

anodization in a sulphuric acid bath;

50 coloring with alternating current in acid solution containing salts of metals of copper, nickel, cobalt and the like, with counter-electrodes made with the constituent metal of the salts or of stainless steel, at current densities within the range of 0.5 to 5 A/dm<sup>2</sup> for a period of time within the range of 1 to 55 15 minutes, to obtain black, red or very deep bronze color effects; and

partial anodic dissolution in the coloring bath.

56 It is preferred, though not essentially a part of the invention, to seal the coating as by 30 minutes' immersion in distilled boiling water containing from 0.5 to 2 g/liter of nickel acetate.

**EXAMPLE 1**

60 A 99.5 percent pure aluminum sheet is mechanically treated to provide a satin surface and then anodized in a sulphuric acid bath to give a porous surface layer of alumina having a thickness of 15 microns. It is then colored by mounting as an electrode in an electrolysis cell fed with alternating current in which the electrolyte is a sulphuric acid solution of copper sulphate having the following composition:

CuSO<sub>4</sub> · 5H<sub>2</sub>O: 20 g/liter

H<sub>2</sub>SO<sub>4</sub>: 5 g/liter

The counter-electrode is made of stainless steel.

65 After 5 minutes of treatment at 0.6 A/dm<sup>2</sup>, a sheet which is dark red in color is obtained.

The cell is then converted to direct current with the sheet mounted as the anode. The sheet is removed after 3 minutes of treatment at 0.2 A/dm<sup>2</sup> at about 20° C.

After sealing in boiling water, a sheet having a clear copper red color is obtained. The color effect is uniform and very dull in appearance and is resistant both to ultra-violet light and to corrosion.

#### EXAMPLE 2

An aluminum sheet containing 0.6 percent magnesium is chemically treated to provide a shiny finish and then anodized in a sulphuric acid bath to obtain a porous layer of alumina having a thickness of 20 microns. It is then mounted as an electrode in an electrolysis cell fed with alternating current in which the electrolyte is a sulphuric acid solution of copper sulphate having the following composition:

$\text{CuSO}_4 \cdot 5\text{H}_2\text{O}$ : 20 g/liter

$\text{H}_2\text{SO}_4$ : 5 g/liter

The counter-electrode is made of copper.

A sheet which is black in color is produced after 10 minutes of treatment at 0.6 A/dm<sup>2</sup>.

The cell is then fed with rectified direct current (unfiltered) with the sheet mounted as the anode. The sheet is removed after 1 minute and 30 seconds treatment at 0.4 A/dm<sup>2</sup> at 20° C.

A sheet which is bright red in color is produced and sealed in boiling water. The color is uniform and brilliant in appearance and resistant to ultra-violet rays and to corrosion.

#### EXAMPLE 3

A section of aluminum alloy containing 0.5% silicon and 0.5% magnesium is mechanically polished and then anodized in a sulphuric bath to provide a surface porous layer of alumina having a thickness of 18 microns. It is then colored by mounting as an electrode in an electrolysis cell fed with alternating current in which the electrolyte is a solution of a mixture of boric acid, nickel sulphate and ammonium sulphate:

nickel sulphate : 100 g/liter

boric acid : 25 g/liter

ammonium sulphate : 30 g/liter

The counter-electrode is made of nickel.

A section which is dark bronze in color is produced after 5 minutes of treatment at 0.4 A/dm<sup>2</sup>.

The section is mounted as the anode and the cell is fed with direct current. The section is removed after 6 minutes of treatment at 0.1 A/dm<sup>2</sup> at 25° C.

After sealing in boiling water, the section has a clear, uniform and brilliant bronze colored finish which is resistant to ultra-violet rays and to corrosion.

#### EXAMPLE 4

An aluminum alloy section containing 1% by weight silicon, 1% by weight magnesium and 1% by weight manganese is cleaned with soda and then anodized in a sulphuric bath to obtain a porous surface layer of alumina having a thickness of 12 microns. It is then colored by mounting as an electrode in an electrolysis cell fed with alternating current, in which the electrolyte is a solution of a mixture of boric acid, cobalt sulphate and ammonium sulphate:

cobalt sulphate : 20 g/liter

boric acid : 25 g/liter

ammonium sulphate : 15 g/liter

The counter-electrode is made of stainless steel.

After 10 minutes of treatment at 0.3 A/dm<sup>2</sup>, the section takes on a dark bronze color.

The cell is then fed with continuous current or direct current with the section mounted as the anode. The section is removed after 4 minutes of treatment at 0.2 A/dm<sup>2</sup> at 20° C.

After sealing in boiling water, the section has a clear, uniform mat bronze color which is resistant to ultra-violet rays and to corrosion.

#### EXAMPLE 5

An aluminum alloy section containing 1% by weight silicon, 1% by weight magnesium and 1% by weight manganese is mechanically polished and then anodized in a sulphuric acid bath to provide a porous surface layer of alumina having a thickness of 15 microns. It is then colored by mounting as an electrode in an electrolysis cell fed with alternating current, in which the electrolyte is a sulphuric acid solution of copper sulphate:

$\text{CuSO}_4 \cdot 5\text{H}_2\text{O}$  : 20 g/liter

$\text{H}_2\text{SO}_4$  : 5 g/liter

The counter-electrode is made of copper.

After 10 minutes of treatment at 0.6 A/dm<sup>2</sup>, the section is black in color.

The cell is then fed with direct current with the section mounted as an anode. The section is removed after 2 minutes of treatment at 20 volts at 20° C.

After sealing in boiling water, the section has a uniform and brilliant copper red finish which is resistant to ultra-violet rays and to corrosion.

It will be apparent from the foregoing that there is provided a new and improved process for producing colored coatings on aluminum and alloys of aluminum in which the colored coating is permanent, resistant to ultra-violet rays, resistant to corrosion, and in which the colored surface is uniform throughout.

It will be understood that changes may be made in the details of formulation and operation without departing from the spirit of the invention, especially as defined in the following claims.

I claim:

1. In a process for color coating objects of aluminum and alloys of aluminum, the steps of anodizing the surface of the object to be colored to produce a porous alumina layer, mounting the object as an electrode in an electrolytic bath containing in solution a salt of a metal which deposits colored particles in the alumina layer in response to alternating current, and passing an alternating current through the bath to deposit colored particles of the metal or a compound of the metal in the porous coating, and then mounting the object as an anode in an electrolytic bath while passing a current therethrough for dissolution of colored particles until the desired color is obtained.

2. The process as claimed in claim 1 which includes the step of sealing the colored coating that is formed.

3. The process as claimed in claim 2 in which the colored coating is sealed with boiling water.

4. The process as claimed in claim 1 in which the current for dissolution is direct current.

5. The process as claimed in claim 1 in which the current for dissolution is rectified unfiltered current.

6. The process as claimed in claim 1 in which the electrolytic bath for the alternating current electrolysis is the same as the electrolytic bath for dissolution so that the object remains in the same bath for both direct current electrolysis and dissolution electrolysis.

7. The process as claimed in claim 6 in which the change from alternating current to direct or rectified current is effected by merely switching from one to the other.

8. The process as claimed in claim 1 which includes the step of subjecting the object to be colored to a surface treatment prior to electrolysis treatment to modify the appearance of the formed colored coating.

9. The process as claimed in claim 1 in which the metal compound deposited in the porous layer contains a compound of copper to produce a color within the range of pink to copper red to bright red.

10. The process as claimed in claim 1 in which the metal compound deposited in the porous layer contains a compound of cobalt to produce a clear bronze color effect in the colored coating.

11. The process as claimed in claim 1 in which the metal compound deposited in the porous layer contains a compound of nickel to produce a uniform clear bronze color effect in the colored coating.

12. The process as claimed in claim 1 in which the current for dissolution has a current density less than 5 A/dm<sup>2</sup>.

13. The process as claimed in claim 1 in which the current for dissolution has a current density within the range of 0.1 to 2 A/dm<sup>2</sup>.

14. The process as claimed in claim 1 in which the current for dissolution is within the range of 10 to 50 volts.

15. The process as claimed in claim 1 in which the current for dissolution is within the range of 15 to 25 volts.

16. The process as claimed in claim 1 in which the dissolution is carried out for a time within the range of 1/6 to 30 minutes.

17. The process as claimed in claim 1 in which the dissolution is carried out for a time within the range of 1/2 to 15 minutes.

18. An object of aluminum or alloy of aluminum having a uniform colored coating produced by the method of claim 1.

\* \* \* \* \*

15

20

25

30

35

40

45

50

55

60

65

70

75